

## UNITED STATES PATENT OFFICE.

CHARLES A. HAMEL, OF SWANTON, VERMONT.

## PUTTY POWDER.

No Drawing.

Application filed April 18, 1923. Serial No. 632,538.

*To all whom it may concern:*

Be it known that I, CHARLES A. HAMEL, a citizen of the United States, residing at Swanton, in the county of Franklin and State of Vermont, have invented certain new and useful Improvements in Putty Powders, of which the following is a specification.

This invention relates to an improved putty powder for use in polishing marble, and the object of the invention is to provide a powder which will be more rapid in its polishing action and will therefore facilitate the work of polishing.

In preparing the putty powder in accordance with the invention, the following ingredients are employed in about the proportions stated:

|                          |         |
|--------------------------|---------|
| French chalk             | 4½ lbs. |
| Oxalic acid              | 1 lb.   |
| Tin oxide                | 1 lb.   |
| Pulverized stone         | 4 lbs.  |
| Chrome oxide (technical) | 1½ lbs. |

The ingredients named above are mixed in the proportions stated and the resulting powdered mixture is then employed both in machine and hand polishing, the same as any other putty powder. However, I have found that a powder of this composition is

more effective in its polishing action and will 30 permit of the work being performed more expeditiously and in a more satisfactory manner than where putty powders of ordinary compositions are employed.

One of the named ingredients is pulverized stone, and with regard to this ingredient it may be said that for this purpose I may employ pulverized marble and preferably a soft white marble. The chalk in the composition constitutes the body or base, 40 and the other ingredients I have found to be highly efficient in both cleansing and polishing the surface of the marble.

Having thus described the invention, what is claimed as new is:

1. A putty powder for marble polishing comprising a mixture of French chalk, oxalic acid, tin oxide, pulverized stone, and chrome oxide.

2. A putty powder for marble polishing comprising a mixture of French chalk, oxalic acid, tin oxide, pulverized stone, and chrome oxide, in about the proportions of French chalk 4½ lbs., oxalic acid 1 lb., tin oxide 1 lb., pulverized stone 4 lbs., and chrome oxide 1½ lbs.

In testimony whereof I affix my signature.

CHARLES A. HAMEL. [L.S.]